

## 1

3,373,117

## LUBRICANTS CONTAINING CHLOROANILINE-PHOSPHATE SALTS

Earl Eugene Sommers, Graylyn Crest, Wilmington, Del., assignor to E. I. du Pont de Nemours and Company, Wilmington, Del., a corporation of Delaware  
No Drawing Filed Dec. 17, 1965, Ser. No. 514,711  
3 Claims. (Cl. 252—32.5)

## ABSTRACT OF THE DISCLOSURE

Salts of aromatic chloroamines and C<sub>8</sub>—C<sub>19</sub> alkyl acid phosphates as extreme pressure additives for conventional lubricating oils and "break-in" lubricating oils.

## Background of the invention

This invention is directed to natural and synthetic lubricating oils having significantly improved antiwear and load carrying ability. These lubricants have incorporated there-in a chlorinated aromatic amine salt of an alkyl acid phosphate.

The need for special lubricant compositions for use in machinery subjected to extreme pressures has long been recognized and is continuing due to constant changes in automotive and industrial equipment. The tendency to reduce the size of power transmitting devices together with increases in engine power have raised the pressures between bearing surfaces so that lubricants having increased load carrying ability are required. Various compounds have been added to lubricants to improve their extreme pressure properties. The use of compounds of chloride, sulfur and/or phosphorus is well known.

Certain organic compounds including some or all of these elements are effective extreme pressure additives. Chlorine containing lubricants are desirable for the reason that under high stress a thin lubricating film is formed, believed to be a metal chloride, between the metal parts. However, incorporation of chlorine into the additive introduces a problem of corrosion, due to the breakdown of the additive under high stress and accompanying increase in temperature, resulting in the formation of corrosive chlorine containing compounds.

## Description of the invention

It is, therefore, an object of this invention to provide a novel lubricant capable of withstanding high contact pressures under severe and adverse operating conditions. It is a further object to provide such a lubricant composition which does not decompose under high stress and increased temperatures to form corrosive compounds, but on the contrary, has intrinsic antirust activity.

These and other objects of the invention will be apparent from the following description and claims.

The present invention is based on the discovery that certain chloroamine salts of acid phosphates have the ability to confer extreme pressure properties to natural and synthetic lubricating oils; said salts do not decompose to form harmful corrosive materials during operation under heavy loads.

The lubricants of the present invention are especially adapted for use in internal combustion engines, industrial gear elements, hydraulically activated systems and similar machinery. These lubricants show improved antirust and antiwear properties. In addition, they have the advantage of being ashless.

More specifically, the present invention is directed to a lubricant composition having improved antiwear and load carrying ability comprising essentially a natural or synthetic lubricating oil and 0.05 to 2.0% by weight of the oil of a salt of an aromatic chloroamine and a C<sub>8</sub>—C<sub>18</sub> alkyl acid phosphate.

## 2

The primary alkyl acid esters of orthophosphoric acid (acid phosphates) which are utilized in the practice of this invention are those esters in which only one or two of the three acidic hydrogen atoms of orthophosphoric acid have been replaced by the alkyl groups, e.g., the monoalkyl dihydrogen phosphates and the dialkyl hydrogen phosphates. Such esters may be obtained according to the general methods of the art which involve reacting an alcohol with phosphorous pentoxide (P<sub>2</sub>O<sub>5</sub>). From about two to about four moles of the alcohol may be used per mole of P<sub>2</sub>O<sub>5</sub>. Preferably, about three moles of the alcohol per mole of P<sub>2</sub>O<sub>5</sub> will be used to yield approximately equimolar mixtures of the mono and dialkyl esters of orthophosphoric acid, containing about 40 to about 60 mole percent of the monoalkyl esters and about 60 to about 40 mole percent of the dialkyl esters. These mixtures of mono- and dialkyl esters are preferred for reasons of economy, but other mixtures, as well as the single monoalkyl esters and single dialkyl esters, may also be used.

For the preparation of these primary alkyl acid phosphates, the alcohol is a branched or straight chain primary alkanol having 8 to 18 carbon atoms or a mixture of two or more straight chain or two or more branched chain alkanols. The branched chain alkanols preferably are those made by the well known oxo process from CO, H<sub>2</sub> and a branched chain olefin such as the C<sub>7</sub>—C<sub>15</sub> monoolefinic polymers and interpolymers of propylene and butylene, as described for example in U.S. Patent 2,824,836, and in U.S. Patent 2,884,379. Examples of preferred oxo-alcohols that may be used are isoctyl alcohol from the propylene-butylene dimer, branched tridecyl primary alcohols from triisobutylene and from tetrapropylene, and the branched hexadecyl primary alcohols from pentapropylene. Other branched chain primary alkanols that can be used are those that may be prepared by alkaline condensation of two primary alkanols, having the structure RCH<sub>2</sub>CH<sub>2</sub>OH wherein R is alkyl and totaling two to six carbon atoms, to produce branched primary alkanols that are branched in the 2-position, i.e.



For example, 2-hexyldecanol-1 is produced by heating n-octanol with caustic and zinc dust, and similarly, 2-ethylhexanol-1 from butanol-1, as described in U.S. Patent 2,457,866. Other alcohols, that may be prepared by the latter and other methods known in the art and used to prepare phosphates according to the present invention, are of the formula RCH<sub>2</sub>CH<sub>2</sub>—CHR—CH<sub>2</sub>OH where R is the same or different alkyl group, each having from two to six carbon atoms. The branched alcohols may also be prepared by the conventional aldolization of suitable aldehydes followed by hydrogenation. In this way, the well known oxo-octaldehyde, which is obtained from heptene-1, CO and H<sub>2</sub> and which is a mixture consisting very largely of dimethylhexaldehydes, ethylhexaldehydes, and methylheptaldehydes containing the grouping



60 is converted into "2-hexyldecanol," R'CH<sub>2</sub>CH<sub>2</sub>OH, where R stands for C<sub>6</sub> alkyl groups, such as dimethylbutyl, methylpentyl and ethylbutyl, and R' stands for C<sub>8</sub> alkyl groups such as dimethylhexyl, ethylhexyl and trimethylpentyl groups. The straight chain primary alkanols are readily available on the market. Examples of such alcohols are octanol, nonanol, decanol, dodecanol, tridecanol, tetradecanol, hexadecanol and octadecanol.

Preferred phosphates are di(2-ethylhexyl)hydrogen phosphate, the mixed mono- and diisoctyl acid phosphates and mixed mono- and di-C<sub>8</sub> to C<sub>16</sub> alkyl acid phosphates. The alkyl radicals of the last named phosphate stem from a mixture of alkanols of average molecular

weight range of 150-155, derived from coconut oil. Hereinafter this phosphate will be referred to as the  $C_8$  to  $C_{16}$  n-alkyl acid phosphate.

The amines used to prepare the salts are the readily available mono- and di-chloro substituted aniline and mono- chloro substituted toluidine. Examples of such amines are o-, m- and p-chloroaniline, 2,4-dichloroaniline, 3,4-dichloroaniline, 3-chloro-o-toluidine and 5-chloro-o-toluidine.

The preferred amines are o-chloroaniline and 3,4-dichloroaniline. The term aromatic chloroamine as utilized herein includes both chloroanilines and chlorotoluidines.

The amine salts of the present invention may be prepared according to any of the methods of the art, by neutralizing the alkyl acid phosphate with the amine. Normally one mole of amine is used for one mole of dialkyl hydrogen phosphate, and two moles of amine for one mole of monoalkyl dihydrogen phosphate. To produce a salt exerting a substantially neutral pH (5-7), about 1.5 moles of amine are required per mole of mixed mono- and dialkyl phosphates.

A representative example of the preparation of the salt follows:

#### EXAMPLE I

53.2 parts (0.2 mol) of mixed (40 to 60%) mono- and (60 to 40%) di-isooctyl acid phosphate and 38.5 parts (0.3 mol) of o-chloroaniline were mixed and heated for one hour at 80° C., then cooled. The resulting product had a total acid number (TAN) of 179.

The additives of the invention may be used with a natural or synthetic lubricating oil. The natural oil may be mineral or vegetable in origin. The mineral oils may be paraffinic, naphthenic or aromatic in nature or a mixture thereof. Examples of such oils are internal combustion engine crankcase oils, gear oils, turbine oils, hydraulic fluids, industrial oils and lubricants. Suitable vegetable oils are castor oil and similar oils.

The synthetic lubricating oils which are also improved are higher molecular weight dicarboxylic acid esters, such as the aliphatic diesters of sebacic, adipic, azelaic, pyromellitic, trimellitic and phthalic acids.

The amount of chloroamine phosphate salt to be added to the lubricating oil base stock is within the range of 0.05 to 2.0 weight percent based on weight of the base oil. The preferred amount is 0.25 to 0.5 weight percent. This amount is effective in markedly improving the extreme pressure and antiwear characteristics of the oil.

The following tests, A through E, illustrate the effectiveness of the chloroamine phosphate salt additive in mineral and synthetic oil.

#### A. Rapid Falex test procedure

The Falex test is described in "Lubricant Testing" by E. G. Ellis, Scientific Publications, Great Britain, 1953, pp. 150-153. The Falex tester consists of a motor driven vertical shaft to which is attached the test pin, which runs between two V-shaped bearing blocks. The tests were conducted for a two-minute wear-in period at 250 pounds jaw load. The eccentric arm was engaged and the jaw load automatically increased to the point of failure. Failure was a result of pin shearing or journal wearthrough.

The Falex test pieces were cleaned just before use by soaking at least 15 minutes in naphtha and then in acetone and finally wiping dry with *clean* cheesecloth. At this point, considerable care must be exercised in order to avoid touching the clean test pieces with contaminated rags, paper, or the fingers. Just prior to inserting the test pieces in the test machine they were examined visually for any obvious surface defects. Any defect was cause for rejection of the test piece.

After the test pieces were inserted in the test apparatus, the loading gear assembly was attached to the lever arms. The sample holder, containing about 55 ml. of the test fluid, was placed in position and the test pieces immersed in the lubricant. Then the load on the bushing-journal

couple was manually adjusted to 250 pounds (jaw load). The machine was then run for two minutes at this jaw load to "break-in" the test pieces. The automatic loading arm was then engaged and the test continued until failure, as indicated by seizure of the test pieces and/or a sharp rise in torque. The jaw load and torque at the instant of failure were noted and recorded for each sample.

The results are listed in Tables I and II wherein a stoichiometric ratio of 1.5 moles of amine to one mole of mixed phosphate was utilized to produce an essentially neutral salt.

TABLE I.—CHLOROAMINE SALTS OF ALKYL ACID PHOSPHATES AS EXTREME-PRESSURE ADDITIVES IN ESTER-LUBRICANT (DI-OXO-TRIDECYL ADIPATE)

|                                                                     | Falex Seizure Test | Maximum Bushing Temp., °F. |       |
|---------------------------------------------------------------------|--------------------|----------------------------|-------|
|                                                                     | Seizure Load, lb.  | Torque at Seizure, lb./in. |       |
| Additives <sup>1</sup> (Base Oil Only)                              | 2,250              | 48                         | ----- |
| Amine Salt of Isooctyl Acid Phosphate: <sup>2</sup>                 |                    |                            |       |
| o-Chloroaniline                                                     | 3,625              | 46                         | 262   |
| m-Chloroaniline                                                     | 3,200              | 45                         | 275   |
| p-Chloroaniline                                                     | 3,750              | 42                         | 252   |
| 2,4-dichloroaniline                                                 | 3,250              | 42                         | 227   |
| 3,4-dichloroaniline                                                 | 3,300              | 46                         | 205   |
| 3-chloro-o-toluidine                                                | 3,450              | 45                         | 242   |
| 5-chloro-o-toluidine                                                | 3,725              | 46                         | 255   |
| Isooctyl Acid Phosphate <sup>2</sup> only                           | 2,350              | 36                         | 230   |
| Amine Salt of $C_8$ - $C_{16}$ n-Alkyl Acid Phosphate: <sup>2</sup> |                    |                            |       |
| o-Chloroaniline                                                     | >4,500             | 44                         | 272   |
| 3-chloro-o-toluidine                                                | >4,500             | 45                         | 230   |
| 3,4-dichloroaniline                                                 | >4,500             | 46                         | 260   |
| $C_8$ - $C_{16}$ n-Alkyl Acid Phosphate <sup>2</sup> only           | 3,770              | 39                         | 268   |
| Amine Salt of di(2-ethylhexyl) hydrogen Phosphate:                  |                    |                            |       |
| 3,4-dichloroaniline                                                 | 3,500              | 50                         | 280   |
| Di(2-ethylhexyl)hydrogen phosphate, only                            | 2,800              | 50                         | 230   |
| Amine Only: 3,4-dichloroaniline                                     | 2,200              | 32                         | 170   |

<sup>1</sup> 2 wt. percent of the additive was blended into the base oil; tests were made on the resultant clear solution.

<sup>2</sup> Phosphate is a mixture of 40-60 mole percent mono- and 60-40% mole percent dialkyl acid phosphates.

Table I.—Esterlube base oils.—Blends of up to 2% of the chloroamine salts of isooctyl acid phosphates in the esterlube base oil permit up to 65% greater load carrying capacity than does a blend of 2% of the isooctyl acid phosphate in the base oil. Similar improvements in load carrying ability are observed with  $C_8$ - $C_{16}$  n-alkyl acid phosphate salts.

TABLE II.—CHLOROAMINE SALTS OF ALKYL ACID PHOSPHATES AS EXTREME PRESSURE ADDITIVES IN WHITE MINERAL OIL (NUJOL)

|                                                                     | Falex Seizure Test | Maximum Bushing Temp., °F. |       |
|---------------------------------------------------------------------|--------------------|----------------------------|-------|
|                                                                     | Seizure Load, lb.  | Torque at Seizure, lb./in. |       |
| Additives <sup>1</sup> (Base Oil Only)                              | 850                | 16                         | 165   |
| Amine Salt of Isooctyl Acid Phosphate: <sup>2</sup>                 |                    |                            |       |
| o-Chloroaniline                                                     | 1,600              | 39                         | 190   |
| m-Chloroaniline                                                     | 2,125              | 40                         | 232   |
| p-Chloroaniline                                                     | 1,975              | 34                         | 275   |
| 2,4-dichloroaniline                                                 | 1,850              | 31                         | 262   |
| 3,4-dichloroaniline                                                 | 2,025              | 35                         | 288   |
| 3-chloro-o-toluidine                                                | 1,700              | 35                         | 200   |
| 5-chloro-o-toluidine                                                | 1,350              | 23                         | 202   |
| Isooctyl acid phosphate only                                        | 1,600              | 28                         | 215   |
| Amine Salt of $C_8$ - $C_{16}$ n-Alkyl Acid Phosphate: <sup>2</sup> |                    |                            |       |
| o-Chloroaniline                                                     | 3,725              | 40                         | 272   |
| 3-chloro-o-toluidine                                                | 3,875              | 48                         | 315   |
| 3,4-dichloroaniline                                                 | 2,525              | 36                         | 220   |
| $C_8$ - $C_{16}$ n-Alkyl Acid Phosphate only                        | 2,575              | 34                         | 247   |
| Amine Salt of Di(2-ethylhexyl) hydrogen Phosphate:                  |                    |                            |       |
| 3,4-dichloroaniline                                                 | 1,450              | 35                         | ----- |
| Di(2-ethylhexyl)hydrogen phosphate only                             | 1,275              | 30                         | ----- |
| Amine Only: 3,4-dichloroaniline                                     | 2,125              | 47                         | 250   |

NOTE.—See footnotes after Table I.

Table II.—White mineral base oil.—Blends of up to 2% of the chloroamine salts of isooctyl acid phosphate carry up to 153% greater load than does the mineral base oil alone and up to 34% greater load than the 2% blends of isooctyl acid phosphate itself; similar benefits are observed for the chloroamine salts of  $C_8$ - $C_{16}$  n-alkyl acid

phosphate salts. These acid phosphates are mixed mono- and di-alkyl phosphates as described herein.

The data for the preceding Tables I and II, and for Tables IV, V, VI and VII are based on a chloroamine salt prepared from 1.5 moles of the chloroamine to one mole of the phosphate.

The following Table III shows the load carrying ability of the o-chloroaniline salt of mixed (40-60 mole percent) mono- and di-isoctyl (60-40%) acid phosphate salt prepared from the varying mole ratios of o-chloroaniline.

TABLE III.—FALEX STEEL ON STEEL SEIZURE TEST  
[2% by weight of additive in di(2-ethylhexyl)sebacate]

|                                                | Seizure Load, lb. | Torque at Seizure, lb./in. | TAN <sup>1</sup> |
|------------------------------------------------|-------------------|----------------------------|------------------|
| o-Chloroaniline Salt of isoctylphosphate:      |                   |                            |                  |
| o-Chloroaniline Salt of isoctyl-phosphate:     |                   |                            |                  |
| 3:1 mole ratio                                 | 3,630             | 44                         | 124              |
| 1.7:1 mole ratio                               | 3,250             | 42                         | 179              |
| 1.5:1 mole ratio                               | 3,525             | 42                         | 179              |
| 3,4-dichloroaniline Salt of isoctyl-phosphate: |                   |                            |                  |
| 1.5:1 mole ratio                               | 3,450             | 47                         | 160              |
| Base Oil Only                                  | 2,610             | 58                         | -----            |

<sup>1</sup> Total acid number.

The negative concentration effect of the chloroamine salts of alkyl acid phosphates is illustrated by the following data from Falex Seizure Test.

|                                                                                     | Falex Seizure Test |                            |  |
|-------------------------------------------------------------------------------------|--------------------|----------------------------|--|
|                                                                                     | Seizure Load, lbs. | Torque at Seizure, lb./in. |  |
| 3,4-dichloroaniline salt of C <sub>8</sub> -C <sub>16</sub> n-Alkyl Acid Phosphate: |                    |                            |  |
| ~2% in Nujol                                                                        | 2,525              | 36                         |  |
| 0.1% in Nujol                                                                       | 4,150              | 48                         |  |
| 5-chloro-o-toluidine salt of mixed mono- and diisoctyl acid phosphate:              |                    |                            |  |
| ~2% in Nujol                                                                        | 1,350              | 28                         |  |
| 0.1% in Nujol                                                                       | 1,775              | 60                         |  |

#### B. Falex constant load wear test

Following the same clean-up procedure described in A, above, the test bushings and test pin were weighed to the nearest 0.1 mg. They were then inserted into the test machine, a "break-in" load of 250 lb. applied and the machine operated with the test lubricant for two minutes. At the end of the "break-in" the load was increased automatically to 1500 lbs. where it was maintained constant for a period of 60 minutes.

At the end of the 60-minute run, the test pieces were removed and cleaned as they were in the initial step. After drying they were reweighed to determine the weight loss in mg. The weight loss of the two test bushings was reported as the sum of both bushings.

TABLE IV.—FALEX CONSTANT LOAD WEAR TEST  
[1500 lb./60 min.]  
Base Oil: Di-oxo-tridecyl Adipate

| Additive Conc., Wt. Percent | Weight Loss, mg.            |                                                     |                        |                                                     |
|-----------------------------|-----------------------------|-----------------------------------------------------|------------------------|-----------------------------------------------------|
|                             | Steel Bushings <sup>1</sup> |                                                     | Steel Pin <sup>2</sup> |                                                     |
|                             | ZDATP <sup>3</sup>          | 3,4-Dichloro Aniline Salt of Isoctyl Acid Phosphate | ZDATP <sup>3</sup>     | 3,4-Dichloro Aniline Salt of Isoctyl Acid Phosphate |
| 2                           | 1.9                         | 6.8                                                 | 3.1                    | 19.5                                                |
| 1                           | 1.2                         | 2.5                                                 | 2.1                    | 9.3                                                 |
| 1/2                         | 1.2                         | 1.4                                                 | 1.5                    | 5.7                                                 |
| 1/4                         | 1.2                         | 0.9                                                 | 1.4                    | 4.7                                                 |
| 1/8                         | 2.6                         | 3.2                                                 | 25.6                   | 3.1                                                 |
| 0                           | Seizure with Base Oil       |                                                     |                        |                                                     |
| 2                           | 1.1                         | 1.6                                                 | 7.4                    | 13.4                                                |
| 1                           | 1.1                         | 1.0                                                 | 56.0                   | 9.5                                                 |
| 1/2                         | ( <sup>3</sup> )            | 0.8                                                 | ( <sup>3</sup> )       | 5.8                                                 |
| 1/4                         |                             | 0.8                                                 |                        | 6.6                                                 |
| 1/8                         |                             | 3.1                                                 | 27.1                   | 70                                                  |
| 0                           | 2.4                         | 8.4                                                 |                        |                                                     |

<sup>1</sup> SAE 4615-4620, 90 min. Rockwell "B", 15 rms. max.

<sup>2</sup> Sanderson Special Drill Rod, 98-102 Rockwell "B", 15 rms. max.

<sup>3</sup> A zinc dialkyldithiophosphate, commercially available from the Lubrizol Corp., normally designated as #1060.

<sup>4</sup> Cast Iron, 15 rms. max.

<sup>5</sup> Excessive wear.

Table IV.—Falex wear test.—The data for the 3,4-dichloroaniline salt of isoctyl acid phosphate are compared with those given by zinc dialkyldithiophosphate, the additive commonly used at the present time.

A typical chloroaniline salt has a negative concentration effect in this wear test. The data in Table IV show that higher wear occurs at 2 wt. percent of the 3,4-dichloroaniline salt of isoctyl acid phosphate than occurs at 1/4 wt. percent in an esterlube base oil. This phenomenon should prove an advantage in "break-in" oils where rapid wear-in of the bearing mating surfaces is desired. As the additive is depleted the wear rate decreases to a normal level. This would obviate the need for a separate "break-in" lubricant followed by an oil change to a conventional lubricant.

#### C. Valve tappet scuffing and wear

Sequence IV (ASTM Special Technical Publication No. 315, American Society for Testing Materials, Philadelphia, Pa., (1962)) describes engine operating conditions likely to require special lubricant characteristics to reduce scuffing and wear of valve tappets under high speed and high temperature operations.

Reference engine and procedure.—Lubricant performance was determined by engine condition at the completion of a series of operations with a reference engine, run on the test stand with appropriate accessories for control of engine temperatures. The definitive operating conditions used with the reference engine are detailed below.

The engine required by the standard procedure is a 1962 Chrysler (361 cu. in. displacement), equipped with standard valve springs and fitted also with supplementary inner valve springs. The springs were adjusted to a 33% overload.

Reference sequence IV—high temperature, high speed—tappet scuffing and wear.—The reference engine was operated at 1200±50 r.p.m. for ten minutes, after which the oil drained, the oil filter changed, and new oil added. Without further warm-up, the engine was operated for two hours under the following conditions:

Speed, r.p.m. 3600±75.  
Load No load.  
Water out temperature, °F. 180±5.  
Oil temperature (in sump), °F. 220±10.

Following this two-hour period, the engine was shut down for two hours, with circulating tap water (35 to 75° F.) being used to cool the engine. This on-and-off operation was repeated for five additional cycles, without initial warm up, after which the camshaft and tappets were removed for inspection.

Duplicate runs were made with the reference engine for better definition of the engine severity level.

Interpretation of engine condition.—On completion of the above sequence of operation, the camshaft and valve tappets were removed for inspection. The condition of the parts was based on visual inspection of the scuffing and wear. Ratings were assigned by use of a reference set of valve tappets.

Supplementary reference engine information.—The reference engine was a normal production 1962 Chrysler V8 (361 cu. in. displacement), equipped with standard valve springs (Part No. 1944854) standard production cam-shaft and pin assembly (Part No. 2268405) and standard tappets (Part No. 2084029). In addition, inner valve springs (Part No. 1555166) were installed. Using suitable spacers, the spring heights were set at 1.860 in. for the outer springs and 1.487 in. for the inner springs, to give a 260-lb. spring load at the valve-open position, which was 33 percent overload.

Some additional spacers were required (about 3/16 in.) to obtain the desired height, 1.487 in., for the inner valve spring.

Engine coolant system.—An external water coolant system was employed to maintain the desired coolant

temperature during engine operation, and to permit cooling the engine during the shutdown portion of each cycle.

*Engine oil coolant system.*—An external heat exchanger, of one-quart capacity, was used to maintain the desired oil temperature.

*Duplicate runs.*—On completion of the first run, the oil was drained, the oil filter removed, and the engine rinsed with flushing oil. A new oil filter, new camshaft, and a new set of tappets were installed. After addition of new oil, the engine was ready for the duplicate run, which followed the same definitive procedure as the first run, including initial warm-up procedure.

TABLE V.—VALVE TAPPET SCUFFING  
[Sequence IV test]

| Base Oil                                                       | Di-oxo-tridecyl Adipate |           | 10W-30 Mineral oil Base |           |
|----------------------------------------------------------------|-------------------------|-----------|-------------------------|-----------|
|                                                                | No. Tappets failed      | Test hrs. | No. Tappets failed      | Test hrs. |
| Additive, Wt. percent:                                         |                         |           |                         |           |
| 0                                                              | 0                       | 12        | 5                       | <1        |
| 2% 3,4-dichloroaniline salt of mixed isoctyl acid phosphate*   | 15                      | <1        | 5                       | 10        |
| 1/2% 3,4-dichloroaniline salt of mixed isoctyl acid phosphate* | 0                       | 12        | —                       | —         |
| 1/4% 3,4-dichloroaniline salt of mixed isoctyl acid phosphate* | 1                       | 12        | 0                       | 12        |
| 2% ZDATP                                                       | 0                       | 12        | 0                       | 12        |

\*1.5 to 1 mole ratio of aniline to acid phosphate.

*Table V.—Valve tappet scuffing.*—The data from this full-scale engine test confirm that obtained in the Falex wear test which showed a negative concentration effect for the 3,4-dichloroaniline salt of isoctyl acid phosphate. At two weight percent in the esterlube base oil, all but one of the tappets failed—performance worse than that of the base esterlube. At 1/4 to 1/2 weight percent additive concentration, only one tappet failed giving performance almost equal to that of two weight percent of ZDATP, the standard type of antiscuffing additive used in most commercial motor oil.

Similar performance was observed in engine tests using this additive in a 10W-30 mineral oil base stock.

#### D. GM single tappet test (defined in Table VI)

This test used a single-cam from a production automotive camshaft. A production valve tappet was spring-loaded against the cam. The tappet load was set at 163 pounds for a ten-minute "break-in," and then the load was increased in 40 pound increments to a maximum load of 600 pounds.

Wear of the tappet surfaces was then determined by a sensitive gauge capable of measuring 1/10000 of an inch.

TABLE VI.—VALVE TAPPET WEAR TEST

[GM Single Tappet Tester]<sup>1</sup>

| Base Oil: White Mineral Oil of Lubricant Viscosity Grade                 | Tappet wear, inches |
|--------------------------------------------------------------------------|---------------------|
| Additive, wt. percent:                                                   |                     |
| 2% 3,4-dichloroaniline salt of mixed isoctyl acid phosphate <sup>2</sup> | 0.0001              |
| 2% ZDATP                                                                 | 0.001               |
| 2% n-octyl pantachloro phenylthio acetate                                | 0.0008              |
| 0.5% nickel dithiodicarbamate                                            | 0.0021              |

<sup>1</sup> "Bench Test Simplifies Search for Better Cam and Tappet Materials," G. H. Robinson, General Motors Engineering Journal, July-August-September 1956, pp. 28-30.

<sup>2</sup> 1.5 to 1 mole ratio of aniline to acid phosphate.

<sup>3</sup> Very clean surface.

*Table VI.—Valve tappet wear test.*—3,4-dichloroaniline salt of isoctyl acid phosphate in a mineral oil base stock, gave significantly lower wear of a steel valve tappet than did the conventionally used additive, zinc dialkyldithiophosphate. The chloroaniline derivative was also superior to a highly chlorinated thioester which the literature reports as a good antiwear agent.

#### E. Dynamic rust test for crankcase lubricants

The test consisted of storing 30 cc. of oil=3 cc. of a synthetic exhaust condensate and a steel specimen in a four-ounce tall-form oil sample bottle in an oven at 140°±5° F. for 24 hours. The synthetic exhaust condensate contained 0.02 weight percent of each of the following chemicals in distilled water: Acetic acid, hydrochloric acid, hydrobromic acid, lead chloride and lead bromide. The metal specimen is 1/8 inch thick 1020 steel, 1/2 inch wide, and six inches long. It was boiled in benzene, sandblasted and then washed in naphtha and dried before placing in the bottle. Fifteen bottles were placed in a special rack inside the oven. The rack was rotated at a speed of 30 r.p.m. The test called for alternating rotation for four hours and nonrotation for four hours for a total time of 24 hours. At the end of the test period the iron specimen was rated for amount of rust according to the following table:

| Percent of area rusted: | Rating |
|-------------------------|--------|
| None                    | 10     |
| 1                       | 9      |
| 5                       | 8      |
| 10                      | 7      |
| 50                      | 5      |
| 100                     | 0      |

TABLE VII.—ANTIRUST PROPERTIES

[Sun-American oven rust test]  
30 ml. Test Sample+3 ml. Exhaust Condensate 140° F., 24 hours

| Additive, <sup>1</sup> Weight Percent                                                   | White Mineral Oil | Ester Lube (Di-oxo-tridecyl Adipate) |
|-----------------------------------------------------------------------------------------|-------------------|--------------------------------------|
| 2% 3-chloro-o-toluidine Salt of Isoctyl Acid Phosphate                                  | 9.7               | 9.7                                  |
| 2% 5-chloro-o-toluidine Salt of Isoctyl Acid Phosphate                                  | 9.7               | 9.5                                  |
| 2% o-chloroaniline Salt of Isoctyl Acid Phosphate                                       | 9.7               | 9.5                                  |
| 40 2% m-chloroaniline Salt of Isoctyl Acid Phosphate                                    | 9.7               | 9.7                                  |
| 2% p-chloroaniline Salt of Isoctyl Acid Phosphate                                       | 9.7               | 9.7                                  |
| 2% 2,4-dichloroaniline Salt of Isoctyl Acid Phosphate                                   | 9.7               | 9.5                                  |
| 2% 3,4-dichloroaniline Salt of Isoctyl Acid Phosphate                                   | 9.7               | 9.8                                  |
| 45 1% 3,4-dichloroaniline Salt of Isoctyl Acid Phosphate                                | —                 | 10                                   |
| 1/2% 3,4-dichloroaniline Salt of Isoctyl Acid Phosphate                                 | —                 | 10                                   |
| 2% 3-chloro-o-toluidine Salt of C <sub>8</sub> -C <sub>16</sub> -n-Alkyl Acid Phosphate | 9.7               | 9.7                                  |
| 50 2% o-chloroaniline Salt of C <sub>8</sub> -C <sub>16</sub> -n-Alkyl Acid Phosphate   | 9.7               | 9.5                                  |
| 2% 3,4-dichloroaniline Salt of C <sub>8</sub> -C <sub>16</sub> -n-Alkyl Acid Phosphate  | —                 | 10.0                                 |
| 2% 3,4-dichloroaniline Salt of di-(2-ethylhexyl)hydrogen phosphate                      | 5.5               | 5.5                                  |
| 2% C <sub>8</sub> -C <sub>16</sub> -n-Alkyl Acid Phosphate                              | 9.7               | 7.4                                  |
| 2% Isoctyl Acid Phosphate                                                               | 6.5               | 8.6                                  |
| 2% Di-(2-ethylhexyl)hydrogen Phosphate <sup>2</sup>                                     | 10.0              | 10.0                                 |
| 55 2% 3,4-dichloroaniline Base Oil Only                                                 | 4                 | 9.2                                  |
|                                                                                         | 5.4               | 5.2                                  |

<sup>1</sup> These salts, except for "+", are essentially neutral salts of the mixed alkyl acid, phosphate; the di-(2-ethylhexyl)-hydrogen phosphate is the di-alkyl.

60 *Table VII.—Antirust properties.*—The aromatic chloroaniline salts of alkyl acid phosphates exhibit good anti-corrosion properties in both mineral and ester base oils. Normally, chlorine is a pro-rust agent and most halogenated extreme pressure or antiwear additives are used where the presence of rust is not serious or can be avoided through other means.

65 The aromatic chloroaniline derivatives are better anti-rust agents than the isoctyl acid phosphate in both the mineral base and the ester base oils. They were also superior to the n-alkyl phosphate in the ester base oil and equal in the mineral base oil. As the data in Table VII indicate, all of the additives were superior to the base oils, themselves. The preceding representative examples may 75 be varied within the scope of the present total specifica-

tion disclosure, as understood and practiced by one skilled in the art, to achieve essentially the same results.

As many apparently widely different embodiments of this invention may be made without departing from the spirit and scope thereof, it is to be understood that this invention is not limited to the specific embodiments thereof except as defined in the appended claims.

The embodiments of the invention in which an exclusive property or privilege is claimed are as follows:

1. A lubricant composition having improved antiwear and load carrying ability, said composition comprising essentially a lubricating oil and 0.05 to 2.0% by weight of the oil of a salt of a chloroaniline selected from the group consisting of orthochloroaniline and 3,4-dichloroaniline and mixed mono- and di-isooctyl acid phosphate.

2. A lubricant composition according to claim 1, said

salt being the ortho-chloroaniline salt of mixed mono- and di-isooctyl acid phosphate.

3. A lubricant composition according to claim 1, said salt being the 3,4-dichloroaniline salt of mixed mono- and di-isooctyl acid phosphate.

#### References Cited

#### UNITED STATES PATENTS

|           |         |               |            |
|-----------|---------|---------------|------------|
| 3,116,248 | 12/1963 | Frew          | 252—32.5   |
| 3,116,249 | 12/1963 | Ratner et al. | 252—32.5   |
| 3,203,895 | 8/1965  | Latos et al.  | 252—32.5   |
| 3,247,109 | 4/1966  | Benoit        | 252—32.5 X |

DANIEL E. WYMAN, *Primary Examiner.*

P. P. GARVIN, *Assistant Examiner.*